

## 1

2,976,238

## OIL-BASED COMPOSITIONS

John Scotchford Elliott and Eric Descamp Edwards, London, England, assignors to Castrol Limited, a British company

No Drawing. Filed Dec. 19, 1957, Ser. No. 703,753

Claims priority, application Great Britain Dec. 24, 1956

8 Claims. (Cl. 252—32.5)

This invention is for improvements in or relating to oil-based compositions and is particularly concerned with lubricating compositions.

It is an object of the present invention to provide lubricating compositions containing additives which additives have a high "alkaline reserve" combined with a relatively low ash content, said lubricating compositions being suitable for use in internal combustion engines.

A further object of the present invention is to provide oil-based compositions having anti-corrosive properties.

It is a still further object of the present invention to provide an improved lubricant for the cylinders of marine diesel engines burning "boiler fuel" or other fuel of high sulphur content.

In our British patent application No. 8,823/55 we have described and claimed a cylinder lubricant for marine diesel engines operating on boiler fuel or other fuel of high sulphur content, which lubricant comprises a mineral lubricating oil having incorporated therein an oil-soluble organic non-aromatic amine having not less than 7 carbon atoms or an oil-soluble non-aromatic amine salt of a weak acid, said organic non-aromatic amine or amine salt being present in an amount sufficient to provide at least 5% of amine in the oil. The non-aromatic amines of this application effectively reduce cylinder wear and improve piston cleanliness of marine diesels operating on boiler fuel, but they suffer from certain disadvantages in that they possess strong odours and have a caustic action on the skin, are prone to cause the removal of paint from surfaces with which they come into contact, and tend to react with carbon dioxide in the atmosphere with the consequent formation of oil-insoluble carbonates or carbamates which form an undesirable skin on the surface. Of the amine salts, on the other hand, those which have adequate oil-solubility, while free from these objections, have rather low neutralisation equivalents which necessitate their use in inconveniently large amounts.

The compositions of the present invention, on the other hand, incorporate oil-soluble compounds of mild odour which compounds are substantially neutral in reaction, yet they have higher neutralisation equivalents and can therefore be used in smaller amounts.

In internal combustion engine oils operating on more conventional fuels, one particular problem in engines operating in cold weather is the so-called "cold sludging" which is due to the ingress of water and fuel combustion products giving rise to the formation of a stiff emulsion or "sludge." Under these conditions of operation, a serious accompaniment of "cold sludging" is the corrosion

## 2

of piston rings and cylinder liners due to the presence of water and acidic products from the combustion of the fuel. The compositions of the present invention employed alone or having incorporated therein conventional detergent and antioxidant additives serve to retard the corrosion of piston rings and cylinder liners under these conditions.

The compositions of the present invention may be employed as lubricants for small two-stroke engines. While conventional mineral lubricating oils may be used for this purpose, the presence of additives to improve piston cleanliness and disperse or soften carbon deposits is often desirable.

The oil-based compositions of the present invention may also be used as storage oils, slushing compositions and general rust-preventing compositions such compositions including, if desired, conventional additives such as metal petroleum (mahogany) sulphonates, wool grease and the like.

15 Certain of the compositions of the present invention may also be employed as lubricants for steam turbines, such lubricants possessing good rust-preventive properties in the presence of water or salt water; conventional antioxidants will also generally be present in such compositions.

20 According to the present invention there is provided an oil-based composition comprising a mineral or synthetic oil having incorporated therein a proportion of a compound having the general formula



wherein M is a polyvalent metal capable of forming ammino co-ordination complexes, A is the residue of an organic acid, B is an organic di- or poly-amine, x and y are small integers satisfying the valency of M and A, z is a small integer such that the co-ordination number of M is partially or completely satisfied, and A and B are selected so that the compound is soluble in the oil.

25 The radical A has preferably one of the following formulae,



or



where R and R' are alkyl, cycloalkyl, aralkyl, alkaryl or aryl groupings, and may carry substituents such as hydroxyl or ester groups or halogen atoms.

30 35 40 45 50 The metal M must be a metal capable of forming relatively stable ammino co-ordination complexes, and is desirably also a metal which is not prone to increase the oxidation rate of the oil in which it is dissolved. The preferred metals are zinc, cadmium, cobalt, tin, lead,

nickel and chromium, although others, such as copper, iron (ferrous), mercury, silver, manganese and the rare or comparatively rare elements of group VIII of the periodic table, e.g. platinum, palladium, ruthenium, osmium or iridium, may be used if desired.

55 60 65 The complex amino compounds employed as the additives in the present invention may be prepared by reacting a salt  $M_x A_y$  with the organic di- or poly-amine.

Examples of suitable salts  $M_x A_y$  are the acetates,

ctoates, laurates, oleates, naphthenates, benzoates, alicylates, petroleum sulphonates, alkylated aryl sulphonates and long chain alkyl and alkylated aryl phosphates.

Examples of the di- or poly-amines B are ethylene diamine, diethylene triamine, triethylene tetramine, tetraethylene pentamine, mixtures of higher polyethylene polyamines, piperazine, p-phenylene diamine and various commercially available long-chain diamines of the general formula R"—NHCH<sub>2</sub>CH<sub>2</sub>CH<sub>2</sub>NH<sub>2</sub> wherein R" represents an alkyl group derived from a fatty acid, e.g. uric acid or from mixed fatty acids obtained from coconut oil, soya bean oil or tallow, these diamines being sold under the registered trademark "Duomeen."

If desired, heterocyclic di- or poly-amines may be employed, examples of suitable compounds being sold under the trademark "Bitran."

It is to be understood that in order to produce oil-soluble compounds it is necessary to select the amine used with reference to the nature of the metal salt with which it is complexed. If, for example, a metal petroleum sulphonate or a naphthenate is used, a wide range of di- or poly-amines may be complexed therewith. If, on the other hand, a salt of a short chain organic acid, e.g. cetic acid, is used, it will be necessary to select a relatively long-chain amine, such as one of the "Duomeens," in order to produce an oil-soluble complex compound.

When the complex ammino compounds are intended to be employed as additives for lubricating oils which are to be subjected to relatively high temperatures, it is necessary to select compounds derived from long-chain di- or poly-amines, since compounds derived, for example, from the polyethylene polyamines tend to decompose with the formation of resinous substances which tend to form objectionable gums on pistons, etc. Thus when, for example, the complex compounds are to be employed in lubricating compositions for I.C. engine oils it is desirable to select those derived from the "Duomeens" or other long-chain di- or poly-amines.

The complex ammino compounds may be prepared by any means known to the art. Thus those made from oil-soluble metal soaps or salts may conveniently be prepared in solution, e.g. in mineral oil, by simply warming with the di- or poly-amine in the appropriate proportions. Generally the molar ratio of amine to metal salt will not exceed 1:1, and it is often advantageous to have slight excess of the metal salt present as this tends to improve the oil-solubility of the product.

When the complex compounds are prepared from oil-insoluble metal salts, a convenient method is to reflux a solution of the di- or poly-amine in petroleum ether or benzene with a slight excess of the salt until the latter passes into solution, after which the solution is cooled and the solvent removed by distillation. Complex compounds of this type are in general readily soluble in hot mineral oil but tend to separate to some extent on cooling. More useful mixed complexes can be prepared by further reacting the oil-insoluble metal salt/amine complex with a proportion of an oil-soluble metal salt in such amounts that the molar ratio of total metal salts to the di- or poly-amine is at least 1:0.8. Specific examples of the oil-soluble complex ammino compounds of the present invention are:

nc naphthenate/diethylene triamine complex (1:0.8 molar ratio)  
 nc acetate/"Duomeen C" complex  
 nc naphthenate/"Duomeen C" complex  
 nc naphthenate/"Bitran P" complex  
 nc oleate/"Duomeen C" complex  
 ead naphthenate/"Duomeen C" complex  
 ead naphthenate/triethylene tetramine complex  
 nc naphthenate/p-phenylene diamine complex

Nickel petroleum sulphonate/"Duomeen C" complex  
 Cadmium octyl phosphate/"Duomeen C" complex

In one form of the present invention the complex ammino compound is of the type described in British patent application No. 39,206/56. Specific examples of complex compounds of this type are:

10 Zinc petroleum sulphonate/triethylene tetramine complex  
 Zinc petroleum sulphonate/tetraethylene pentamine complex  
 Tin petroleum sulphonate/triethylene tetramine complex

15 Alternatively, complex compounds may be prepared from certain commercially available materials having a relatively high organic acidity, e.g. crude wool grease. These may be neutralised directly with a suitable metal oxide or hydroxide, e.g. zinc oxide, and then complexed with the desired amine.

20 It is to be understood that the foregoing examples are merely illustrative of the complex compounds which may be employed and are in no wise to be regarded as limiting the scope of the invention. The following remarks may, however, serve to indicate the scope and 25 limitations of different sub-classes of the complex compounds intended for use in the compositions of the present invention.

25 The most generally useful complex compounds are those prepared from freely oil-soluble metal salts e.g. the 30 laurates, oleates and, particularly, the naphthenates of metals such as zinc, nickel, cobalt, tin and chromium and long-chain diamines, particularly the "Duomeens." As already indicated, the "Duomeens" have the general formula R"—NHCH<sub>2</sub>CH<sub>2</sub>CH<sub>2</sub>NH<sub>2</sub>, the radical R" being 35 derived from a fatty acid, and substances are commercially available in which R" is derived from coconut fatty acids ("Duomeen C"), soya fatty acids ("Duomeen S") and tallow fatty acids ("Duomeen T"). Any of these substances may be employed in the production of 40 the complex compounds, but it is generally preferred to use "Duomeen C" as this substance has the best oil-solubility and the highest neutralisation equivalent. Zinc is generally the preferred metal both for economic reasons and because the zinc salts of organic acids can 45 readily be prepared by direct neutralisation of the acids with zinc oxide in the presence of a little water. To obtain the maximum oil-solubility, particularly at low temperatures, it is generally desirable to have a small excess of the metal salt present, a molar ratio of salt:amine of 50 1:0.8 being particularly suitable. Complex compounds of this general type are suitable for use in a variety of lubricating compositions in accordance with the present invention. Thus quite large amounts, up to about 30% by weight, may be used in cylinder oils for marine diesel 55 engines burning boiler fuel, while quite small amounts e.g. 0.2% or less, are effective corrosion inhibitors when used in steam turbine oils, and they do not increase to an unacceptable degree the demulsification values of such oils.

60 Complex compounds having adequate oil-solubility may also be prepared from freely oil-soluble metal salts, e.g. zinc naphthenate, and diethylene triamine or other polyethylene polyamines. These may be used equally well as corrosion inhibitors in steam turbine oils, but as already indicated their use should not be considered in lubricants liable to be subjected to relatively high temperatures.

65 Complex compounds prepared from metal petroleum sulphonates or the metal salts of synthetic oil-soluble alkylated aromatic sulphonates are also freely oil-soluble when prepared from the "Duomeens" and satisfactorily oil-soluble materials can be made from other amines as well. These compounds are good corrosion inhibitors 70 but tend to act also as emulsifiers and their use in turbine

oils is therefore contra-indicated. These compounds, like those derived from the metal salts of organic phosphoric acids, possess a lower reserve alkalinity than those derived from metal carboxylates because the organic sulphonate and phosphoric acids are strong acids not readily displaced from combination with the metal.

Complex compounds prepared from aromatic or heterocyclic di- or poly-amines such as p-phenylene diamine and the "Bitrans" are in general less satisfactory as corrosion inhibitors than the classes already described.

The additives of the present invention may be employed, if desired, in conjunction with other additives commonly used in lubricating oils. Thus, for example, in oils for internal combustion engines there may be present conventional detergents such as metal petroleum (mahogany) sulphonates, and antioxidants such as zinc dialkyl dithiophosphates, metal alkyl phenol sulphides or phosphorised sulphurised terpenes.

The additives may be employed not only in mineral lubricating oils but also in synthetic oils, e.g. the dicarboxylic acid diester type and the polyglycol ether type of synthetic lubricant.

When the oil-based compositions of the present invention are employed as lubricants for the cylinders of marine diesel engines operating on boiler fuel or other fuel of high sulphur content they may contain from 2 percent to 20 percent by weight of the complex amino compound. For use in the lubrication of internal combustion engines using more conventional fuels the additive is preferably used in a proportion of from 0.5 to 2 percent.

For use in turbine oils, selected additives may be used in concentrations ranging from 0.02% to 2.0% and preferably from 0.05% to 0.2%. In general rust-preventive compositions the additives may be employed in widely differing amounts depending on the application which is in mind; thus from about 0.1% up to 10% or even 20% may be used depending on the severity of the conditions.

The following examples illustrate the preparation and properties of the complex compounds which may be used in the lubricating compositions of the present invention:

#### EXAMPLE 1

##### *Zinc naphthenate diethylene triamine complex (Compound A)*

To 709 grams (0.55 mol) of an approximately 50% solution of zinc naphthenate in mineral oil were added 51.5 grams (0.5 mol) of diethylene triamine. An exothermic reaction took place, following which the material was stirred at 110° C. for 15 minutes. The product was a brown oil containing 4.8% zinc and 2.7% nitrogen, and was freely soluble in mineral oil although diethylene triamine itself was quite insoluble.

The "reserve alkalinity" of this complex compound was found to be 176 mgs. KOH per gram, the "reserve alkalinity" of the original zinc naphthenate concentrate being about 80 mgs. KOH per gram.

"Reserve alkalinity" was determined by refluxing a weighed quantity of the sample with a known excess of 0.1 N HCl in a solution consisting of

5% methanol  
45% ethanol  
50% water

and back-titrating with 0.1 N NaOH using screened methyl orange as indicator.

#### EXAMPLE 2

##### *Zinc naphthenate "Duomeen C" complex (Compound B)*

A mixture of 1911 grams (1.5 mols) of an approxi-

mately 50% solution of zinc naphthenate in mineral oil and 300 grams (1.2 mols) of "Duomeen C" were heated to 120° C. and stirred for a few minutes until a bright clear product was obtained.

The product was freely miscible with mineral oil although the oil-solubility of "Duomeen C" itself was very limited. It contained 4.3% zinc and had a "reserve alkalinity" of about 110.

10

#### EXAMPLE 3

##### *Zinc acetate "Duomeen C" complex*

To a solution of 32.1 grams (0.13 mol) of "Duomeen C" dissolved in 200 mls. of toluene were added 18.35 grams (0.10 mol) of anhydrous zinc acetate and the mixture was refluxed until virtually all the zinc acetate had passed into solution. After filtering from a little solid matter, the toluene was removed by distillation in vacuo. The product contained 13.6% zinc and had a "reserve alkalinity" of about 550 mgs. KOH per gm. It was readily soluble in hot mineral oil but some separation occurred on cooling.

25

#### EXAMPLE 4

##### *Zinc acetate-naphthenate "Duomeen C" complex (1:0.5:1 molar ratio)*

A mixture of 18.35 gms. (0.1 mol) of anhydrous zinc acetate and 25.0 gms. (0.1 mol) of "Duomeen C" were stirred together in a beaker and heated slowly to 130° C. Most of the zinc acetate appeared to react in the temperature range 100 to 120° C. yielding a buff opaque viscous liquid. 53.6 grams (0.05 mol) of an approximately 50% oil solution of zinc naphthenate was now added and heating and stirring continued for a few minutes. The zinc naphthenate employed contained 12% zinc. The product was mixed with filter-aid and filtered hot. On dilution with an equal weight of mineral oil a clear stable 36% oil concentrate was obtained containing 5.2% of zinc and having a "reserve alkalinity" of about 130 mgs. KOH per gram.

40

#### EXAMPLE 5

##### *Zinc salt of crude wool grease "Duomeen C" complex (Compound C)*

To 256 gms. (0.2 mol) of a crude wool grease, containing free acidity corresponding to an equivalent weight of 1278, was added 10 gms. of zinc oxide made into a paste with water. The mixture was thoroughly stirred at 90° C. until the zinc oxide had largely reacted, after which the product was heated to 150° C. to remove water.

To 100 gms. (0.038 mol) of this product, held at 90° C., were added 7.9 gms. (0.032 mol) of "Duomeen C." An exothermic reaction took place and the mixture was then heated with stirring until the temperature reached 120° C.

The product was a dark brown solid containing 3.04% zinc.

By the general procedure outlined above, a large number of complex compounds suitable for use in the oil-based compositions of the present invention, may be prepared. The direct heating method of Examples 1 and 2 is generally the preferred method, but various compounds derived from oil-insoluble metal salts, e.g. zinc benzoate, zinc salicylate, may be made by the method of Example 3.

Details of those compounds used in the tests which follow are listed in Table I:

7  
TABLE I

| Complex Compound                                            | Approximate Molar ratio of salt:amine | Approximate Reserve Alkalinity (Mgs. KOH/gm.) |
|-------------------------------------------------------------|---------------------------------------|-----------------------------------------------|
| Compound D, Lead naphthenate-triethylene tetramine complex  | 1:0.8                                 | 320                                           |
| Compound E, Nickel petroleum sulphonate "Duomeen C" complex | 1:1                                   | 80                                            |
| Compound F, Zinc oleate "Duomeen C" complex                 | 1:0.85                                | 230                                           |
| Compound G, Lead naphthenate "Duomeen C" complex            | 1:1.1                                 | 300                                           |
| Compound H, Zinc naphthenate "Bitran P" complex             | 1:1.1                                 | 220                                           |
| Compound I, Chromium caproate "Duomeen C" complex           | 1:0.8                                 | 210                                           |
| Compound J, Cobalt stearate "Duomeen C" complex             | 1:0.9                                 | 205                                           |

Where the composition of the di- or poly-amine was not known with certainty, the amount to be complexed with the metal salt was calculated from a determination of the basicity of the amine.

In order to demonstrate the anticorrosive properties of certain of the oil-based compositions of the present invention, the additives were dissolved in a typical steam turbine base oil consisting of approximately 80% by weight mineral oil "A" and 20% by weight mineral oil "B," and examined for effect on demulsification number and rust preventive characteristics in the presence of salt water. The methods of test employed were those described in "Standard Methods for Testing Petroleum and Products" (16th Edition, February 1957), serial designations I.P. 19/55 and I.P. 135/56 respectively. The results of a series of tests are summarized in Table II.

TABLE II

| Test No.   | Additive | Percent by weight in oil | Demulsification Number | Results of 24 hours salt-water corrosion test at 140° F. |
|------------|----------|--------------------------|------------------------|----------------------------------------------------------|
| None       |          |                          | 60                     | Severe rusting.                                          |
| Compound A | 0.2      |                          | 180                    | No rusting.                                              |
| Compound B | 2.0      |                          | 300                    | Do.                                                      |
| do         | 0.1      |                          | 240                    | Do.                                                      |
| Compound C | 0.2      |                          | over 1200              | Do.                                                      |
| Compound D | 0.2      |                          | 270                    | Do.                                                      |
| Compound E | 0.2      |                          | 720                    | Do.                                                      |
| Compound F | 0.2      |                          | 570                    | Do.                                                      |
| Compound G | 0.2      |                          | 390                    | Do.                                                      |
| Compound H | 1.0      |                          | 75                     | Moderate rusting.                                        |
| Compound I | 0.2      |                          | 150                    | Very slight rusting.                                     |
| Compound J | 0.2      |                          | 150                    | No rusting.                                              |

In mineral oil "B" (demulsification No. 30).

Oil "A" was a mineral oil having a viscosity of about 100 seconds Redwood I at 140° F. and oil "B" was a solvent-refined oil of viscosity about 65 seconds Redwood at 140° F.

It will be seen that while many of the additives tested are effective inhibitors of corrosion under the conditions of this test, some, particularly compounds C and E, increased the demulsification number of the oil to an undesirable extent and therefore were not suitable for use in turbine oils.

Representative oil-based compositions of the present invention were subjected to a very severe test applicable to anticorrosive engine lubricating oils designed to protect aero-engines from corrosion during storage and shipment overseas.

The test procedure is described in Ministry of Defence Specification DEF 2181, Appendix B (issued March 13, 1953) and involved immersion of mild steel panels in a

8  
solution of hydrobromic acid in kerosine followed by immersion in the oil composition, diluted with petroleum ether, followed by draining and maintenance at 20° C. ± 2° C. for 24 hours in a glass vessel over saturated zinc sulphate solution. Protection against corrosion was considered adequate if the average weight gain of the test panels (tested in quadruplicate) did not exceed 5 mgs. Results of these tests are summarized in Table III.

TABLE III  
[All compositions were based on mineral oil "C"]

| Test No. | Additives Present, Percent by weight                                               | Average weight gain (mgs.) |
|----------|------------------------------------------------------------------------------------|----------------------------|
| 13       | 5% Compound B, 4% Sodium petroleum sulphonate soln. (approx. 45% oil concentrate). | 5.5                        |
| 14       | 10% Compound C                                                                     | 10.8                       |
| 15       | 5% Compound C, 4% Sodium petroleum sulphonate soln. (approx. 45% oil concentrate). | 4.8                        |
| 16       | 10% Compound D                                                                     | 4.95                       |

25

Mineral oil "C" was a conventionally refined paraffinic brightstock of viscosity about 600 seconds Redwood I at 140° F.

It will be seen from the foregoing table that 10% of Compound D gave satisfactory protection against corrosion, but that 10% of Compound C was inadequate. Satisfactory protection could, however, be obtained by the use of mixtures of Compounds B or C with sodium petroleum sulphonates.

In order to assess the effectiveness of certain of the oil-based compositions of the present invention as cylinder lubricants for marine diesel engines operating on boiler fuel, engine tests were carried out in a two-cylinder Lister engine (model 12-2, bore 4½", stroke 5½") modified for separate mechanical lubrication of one cylinder.

This engine was operated under the following conditions:

|    |                          |                      |
|----|--------------------------|----------------------|
| 45 | Speed                    | 700 r.p.m.           |
| 50 | B.H.P.                   | 8.                   |
|    | Sump temperature         | 125 ± 5° F.          |
|    | Water outlet temperature | 115 ± 2° F.          |
|    | Water inlet temperature  | 108° F. approx.      |
| 55 | Fuel:                    |                      |
|    | 50% boiler fuel          |                      |
|    | 50% gas oil-1% sulfur    | Sulfur content 2.0%. |

60 No. 1 cylinder was lubricated mechanically, the rate of feed of the test oil to this cylinder being 20 cc. per hour per lubricator i.e. 40 cc. per hour total. No. 2 cylinder was lubricated normally with oil from the sump.

In the tests, details of which are tabulated in Table IV the base oil (mineral oil "D") was used throughout in the sump while various lubricants prepared in accordance with the present invention were used for lubricating No. 1 cylinder. Since these lubricants were all based on mineral oil "D" a direct measure of the effectiveness of the additives could be obtained in any one test by comparing the wear of the two cylinders and cleanliness of the two pistons.

65 Mineral oil "D" was a solvent-refined mineral oil of viscosity approximately 170 seconds Redwood I at 140° F.

70

75

TABLE IV.—LISTER ENGINE TESTS

| Test No. | Lubricant Composition (Cylinder No. 1)                                                                        | Test duration (hours) | Cylinder No. | Top ring wt. loss (mgs.) | Total ring wt. loss (mgs.) | Piston Rating |            |                     |
|----------|---------------------------------------------------------------------------------------------------------------|-----------------------|--------------|--------------------------|----------------------------|---------------|------------|---------------------|
|          |                                                                                                               |                       |              |                          |                            | Skirt         | Lands      | Ring groove lacquer |
| 17       | Mineral Oil "D"                                                                                               | 50                    | { 1<br>2     | 113<br>113               | 229<br>245                 | 29.4<br>29.2  | 4.6<br>4.7 | 1.6<br>1.3          |
| 18       | 93.5% Mineral Oil "D"<br>5.0% Basic barium petroleum sulphonate soln.<br>(approx. 45% in mineral oil)         | 44                    | { 1<br>2     | 174<br>172               | 310<br>317                 | 29.5<br>29.0  | 6.9<br>7.3 | -----               |
| 19       | 1.5% Zinc dihexyl dithiophosphate soln. (approx.<br>50% in mineral oil)<br>91% Mineral Oil D<br>8% Compound B | 96                    | { 1<br>2     | 73<br>290                | 161<br>522                 | 30.0<br>26.3  | 9.9<br>3.2 | 7.6<br>0            |
| 20       | 1% Basic barium petroleum sulphonate soln. (ap-<br>prox. 45% in mineral oil)<br>As test No. 19                | 100                   | { 1<br>2     | 74<br>381                | 111<br>660                 | 30.0<br>27.5  | 9.9<br>4.9 | 7.9<br>0.2          |

Maximum rating for piston skirt..... 30.0  
Maximum rating for piston lands..... 10.0  
Maximum rating for ring groove lacquer..... 10.0

These maximum figures were arbitrary ratings signifying that the parts concerned were perfectly clean. A minimum rating of 0 would be given for a completely black piston or for lands or grooves completely coated with black lacquer.

It will be seen from the foregoing table that although some variation in piston ring weight loss was experienced using the same base oil in different tests, a typical composition of the present invention (tests Nos. 19 and 20) produced a very substantial reduction in wear as compared with the base oil, this being coupled with a marked increase in piston cleanliness. When both cylinders were lubricated with the base oil (test No. 17) there was no significant difference between the two pistons. When a conventional heavy duty oil containing additives in "Supplement 1" proportions was used (test No. 18) it showed no noticeable improvement over the base oil.

A further series of tests were carried out in a Petter AV-1 engine operating under the following conditions:

Test duration ..... hours 100  
Speed ..... r.p.m. 1500  
B.H.P. ..... 5

Engine water-cooled, with normal flow.  
Sump temperature ..... ° F. 158±5  
Water outlet temp. ..... ° F. 149±2  
Water inlet temp. ..... ° F. 131±2

The fuel used was the same as that used in the Lister engine tests. Results of the tests are summarized in Table V.

TABLE V.—PETTER ENGINE TESTS

| Test No.                                   | 21                        | 22                          | 23                                                                                                          | 24                                                                                                               |
|--------------------------------------------|---------------------------|-----------------------------|-------------------------------------------------------------------------------------------------------------|------------------------------------------------------------------------------------------------------------------|
| Lubricant Composition                      | Oil D                     | 90% Oil D<br>10% Compound A | 91% Oil D<br>8% Compound B<br>1% Basic barium pe-<br>troleum sulpho-<br>nate soln. (approx.<br>45% in oil). | 74% Oil D.<br>25% Compound "B."<br>1% Basic barium pe-<br>troleum sulpho-<br>nate soln. (approx.<br>45% in oil). |
|                                            | Maximum rating obtainable |                             |                                                                                                             |                                                                                                                  |
|                                            | Test Result               |                             |                                                                                                             |                                                                                                                  |
| Crown cutting rating                       | 5.0                       | 3.9                         | 3.6                                                                                                         | 4.1                                                                                                              |
| General components rating                  | 10.0                      | 4.1                         | 3.7                                                                                                         | 5.1                                                                                                              |
| Scraper ring sludge rating                 | 10.0                      | 9.0                         | 7.5                                                                                                         | 10.0                                                                                                             |
| Piston lands rating                        | 10.0                      | 0.6                         | 0.0                                                                                                         | 5.3                                                                                                              |
| Piston skirt rating                        | 30.0                      | 22.3                        | 28.2                                                                                                        | 29.2                                                                                                             |
| Ring sticking rating                       | 35.0                      | 28.0                        | 11.7                                                                                                        | 35.0                                                                                                             |
| Top ring groove carbon rating              | 10.0                      | 0.9                         | 0.0                                                                                                         | 5.1                                                                                                              |
| Total ring weight loss <sup>1</sup> (mgs.) | 892                       | 459                         | 419                                                                                                         | 261                                                                                                              |
|                                            | 1,475                     | 745                         | 623                                                                                                         | 464                                                                                                              |

<sup>1</sup> Relates to combined weight loss of 5 rings except in Test No. 22 where only 4 rings were used.

It will be seen from this table that typical compositions of the present invention (tests Nos. 22 to 24) effected a substantial reduction in piston ring corrosion as compared with the plain mineral oil (test No. 21). Compositions containing Compound B, however, were much superior to that containing compound A with respect to

70 and  
75 where R and R' are selected from the group consisting



f alkyl, cycloalkyl, aralkyl and aryl groups; and B is long-chain diamine having a general formula



where  $R''$  is an alkyl group having from 8 to 18 carbon atoms;  $x$  and  $y$  are small integers satisfying the valency requirements of M and A, and  $z$  is a small integer such that the coordination number of M is at least partially satisfied.

2. A composition as claimed in claim 1 wherein the lubricating oil is a mineral oil.

3. A composition as claimed in claim 1 wherein the lubricating oil is selected from the group consisting of carboxylic acid diester oils and polyglycol ether oils.

4. A composition as claimed in claim 1 wherein the complex amino compound is a complex consisting of inc naphthenate/ $R''-\text{NHCH}_2\text{CH}_2\text{CH}_2\text{NH}_2$  wherein  $R''$  is an alkyl group having from 8 to 18 carbon atoms.

5. A composition as claimed in claim 1 wherein the complex amino compound is a complex consisting of inc oleate/ $R''-\text{NHCH}_2\text{CH}_2\text{CH}_2\text{NH}_2$  wherein  $R''$  is an alkyl group having from 8 to 18 atoms.

6. A composition as claimed in claim 1 wherein the complex amino compound is a complex consisting of inc naphthenate/ $R''-\text{NHCH}_2\text{CH}_2\text{CH}_2\text{NH}_2$  wherein  $R''$  is an alkyl group having from 8 to 18 carbon atoms.

7. A composition as claimed in claim 1 wherein there

is present from 5 to 30 percent by weight of the oil-soluble complex amino compound.

8. A cylinder lubricant for marine diesels operating on fuel of high sulphur content consisting essentially of a mineral oil having incorporated therein from 2 to 30 percent by weight of an oil-soluble complex amino compound consisting of



10 having a molar ratio of metal salt to the diamine of at least 1:0.8, wherein  $R''$  is an alkyl group having from 8 to 18 carbon atoms.

#### References Cited in the file of this patent

##### UNITED STATES PATENTS

|           |                     |                |
|-----------|---------------------|----------------|
| 2,684,292 | Caron et al. -----  | July 20, 1954  |
| 2,692,858 | Evans et al. -----  | Oct. 26, 1954  |
| 2,696,473 | Sokol -----         | Dec. 7, 1954   |
| 2,736,658 | Pfohl et al. -----  | Feb. 28, 1956  |
| 2,737,492 | Beegle et al. ----- | Mar. 6, 1956   |
| 2,752,311 | McCoy et al. -----  | June 26, 1956  |
| 2,798,045 | Buck et al. -----   | July 2, 1957   |
| 2,805,996 | Deger -----         | Sept. 10, 1957 |
| 2,808,376 | Lowe -----          | Oct. 1, 1957   |

##### FOREIGN PATENTS

|         |                     |               |
|---------|---------------------|---------------|
| 696,064 | Great Britain ----- | Aug. 26, 1953 |
|---------|---------------------|---------------|